

# United States Patent Office.

JOHN HASELTINE, OF WARREN, NEW HAMPSHIRE.

*Letters Patent No. 67,760, dated August 13, 1867.*

## IMPROVED COMPOSITION FOR STUFFING LEATHER BELTS.

The Schedule referred to in these Letters Patent and making part of the same.

TO ALL WHOM IT MAY CONCERN:

Be it known that I, JOHN HASELTINE, of Warren, in the county of Grafton, and State of New Hampshire, have invented a new and improved Composition for Stuffing the Leather Belts which are used for driving machinery and for rendering such belts more adhesive; and I hereby declare that the following is a full, clear, and exact description of the method of compounding and using the same, and the proportions of the ingredients, specimens of which, as also of the composition, accompany this application.

Recent experiments have demonstrated that the leather belts which are used for driving machinery will endure much longer and perform better service if that portion or side of the belt next the pulleys, or the surface of such leather, and for a short distance in, is filled or stuffed with some suitable substance which will make the leather limber and pliable, and at the same time as adhesive as possible. It is also important that when once prepared, such belts should retain their pliable and adhesive character for a long time.

To accomplish all this the composition used for stuffing or preparing the leather or the belt should contain certain peculiar properties for preserving and softening the leather, and for attracting or drawing moisture from the surrounding atmosphere, as well as for making the belt adhesive, as that portion or property which attracts the moisture aids materially in maintaining and preserving the adhesive property of the composition.

In preparing my improved composition for stuffing and rendering leather belts adhesive, I take as a base for said composition, and for a certain quantity, about one gallon of soap in a semi-liquid state, say about the consistency of common soft soap. To this I add about two pounds of fatty oil or grease, placing the same in a suitable vessel over a slow fire or moderate heat, and stir or agitate till well mixed together. I then add about one pint of common tar, known as North Carolina or Wilmington tar. I also add about one-half pint of common salt, stirring or agitating till the whole mass is well mixed or incorporated, when the composition is ready for use, or it may be allowed to cool before being used.

This composition may be applied to the belt with a brush or a cloth, or with the hand, and well worked into the leather. The effect of this improved composition is as follows: The alkali in the soap has a tendency to soften the leather, the grease contained in the soap and the grease or fatty oil added tend also to soften and to preserve the leather. The tar will remain on the surface and render the leather or belt adhesive, and the salt is partly absorbed by the leather, but most of the salt is retained on the surface, and with the tar the salt attracts or draws moisture from the surrounding atmosphere and keeps the composition and the surface of the belt in an adhesive condition for a very great length of time.

It has been generally supposed that soap has an injurious effect upon leather, but I find it otherwise, and when combined with other ingredients, as above stated, the composition is very beneficial to the leather, as it keeps it soft, limber, and pliable, and prevents other and injurious substances or matter which may come in contact with the belt from having any injurious effect upon it.

Soap may be made for the base of my improved composition with more than the ordinary quantity of grease, and such soap made to serve the purpose of the soap and grease or fatty oil above named, but, as will be readily seen, such soap would be of no use for other purposes, as soap is designed for removing grease from textile fabrics or other substances.

Having fully described my invention, its nature, effect, and the method of compounding, what I claim as of my invention, and desire to secure by Letters Patent, is—

I claim the combination of the ingredients above named, in about the proportions specified, using as a base for my composition the first-named ingredient.

JOHN HASELTINE.

Witnesses:

JOHN E. CRANE,  
J. S. WHITNEY.